

## UNITED STATES PATENT OFFICE

2,212,628

## DYEING MIXED FABRICS

Hermann Winkeler, Ludwigshafen - on - the - Rhine, Germany, assignor to General Aniline & Film Corporation, a corporation of Delaware

No Drawing. Application September 24, 1937, Serial No. 165,511. In Germany October 10, 1936

4 Claims. (Cl. 8—22)

The present invention relates to an improved method of dyeing mixed fabrics.

When dyeing mixed fabrics of animal and vegetable fibres, such as mixed fabrics of wool with cotton or regenerated cellulose, attempts are frequently made to increase the fastness properties of the dyeings, especially their fastness to moisture, by treatment with chromates or bichromates, as for example by the action of alkali bichromates and acetic acid. A process which is especially easily carried out in practice and therefore frequently employed is the so-called "half-wool metachrome process" according to which the dyeing is carried out in the presence of ammonium sulphate and alkali metal chromate. In this case either substantive dyestuffs capable of being chromed and which are equally well taken up by animal and vegetable fibres are used or mixtures of substantive dyestuffs with wool dyestuffs capable of being chromed and which dye only the wool in the mixed fabric.

There is no fundamental difference between the two said dyeing processes; the chromates and bichromates are reduced to salts of trivalent chromium to which the chroming action is due. In both cases the wool portion of the mixed fabrics is dyed sufficiently fast, but the dyeings on the vegetable portion of the mixed fabrics have only an insufficient fastness to water.

I have now found that when dyeing mixed fabrics of animal and vegetable fibres with substantive dyestuffs capable of being chromed or with mixtures of such dyestuffs with wool dyestuffs capable of being chromed especially valuable dyeings are obtained when using besides a chromate or a bichromate at any stage of the dyeing process salts of trivalent chromium. The treatment may be carried out, for example, by dyeing the mixed fabric with the said dyestuffs, converting them into the complex chromium compounds either by an after treatment with a chromate or a bichromate, or according to the "half-wool metachrome process," and then allowing a salt of trivalent chromium to act on the fabric thus treated, in a second bath. It is also possible to treat the fibre dyed with the said dyestuffs in a separate bath with a chromate or bichromate and simultaneously with a salt of trivalent chromium. Finally, the procedure may consist in treating the fibre in the same bath with the said dyestuffs and a salt of chromic acid, adding a salt of trivalent chromium towards the end of the treatment. In the last case, it is preferable to use, for rinsing the dyeing, hot water to which has been added soap or another wetting or dispersing agent.

Among chromium salts suitable for the proposed treatment there may be mentioned for example the fluoride, sulphate, formate, acetate,

oxalate of trivalent chromium or mixtures of the said salts.

The improvement of the fastness to water, i. e. the fastness to water, washing, fulling, sea water and perspiration, by the treatment with salts of trivalent chromium takes place especially readily in the case of dyestuffs in which salicylic acid groups are present in the molecule; ortho-carboxy-hydroxyazo dyestuffs and many ortho-hydroxyazo dyestuffs may also be dyed well on mixed fabrics according to this invention.

The following examples will further illustrate how my said invention may be carried out in practice but the invention is not restricted to these examples.

## Example 1

A mixed fabric of 70 per cent of wool and 30 per cent of viscose artificial silk is dyed in a 20 bath with a bath ratio of 1:40 with 3 per cent of the azo dyestuff derived from 1 molecular proportion of tetrazotized 4,4'-diaminodiphenyl urea and 2 molecular proportions of salicylic acid with an addition of 1 per cent of sodium chromate and 2 per cent of ammonium sulphate in the following manner: the bath is brought during the course of half an hour to 90° C., kept for 1½ hours at the said temperature and the fabric allowed to remain in the cooling bath for an 30 hour. Both kinds of fibre are thus dyed rather uniformly in greenish yellow shades which have a moderate fastness to moisture. The dyed fabric is then treated for half an hour with 2 per cent of chromic sulphate or chromic formate 35 (calculated with reference to the weight of the fabric), the fastness properties thus being improved to an extraordinary extent.

A fabric dyed in an equally fast manner may also be obtained by adding chromic formate to 40 the dyebath towards the end of the dyeing process and shortly soaping the dyeing at about 40° C.

## Example 2

A mixed fabric of 30 per cent of wool and 70 45 per cent of viscose artificial silk is dyed in the manner described in Example 1 with the dyestuff derived from 1 molecular proportion of tetrazotized 4,4'-diaminodiphenyl-3,3'-dicarboxylic acid, 1 molecular proportion of 1-hydroxy-naphthalene-5-sulphonic acid and 1 molecular proportion of 2-phenylamino-5-hydroxynaphthalene-7-sulphonic acid (coupled alkaline). In this way violet shades are obtained which have a slight fastness to washing and water. By after-treating the dyed fabric for half an hour with 2 per cent of chromic sulphate (calculated with reference to the weight of fabric), dyeings having considerably improved fastness to washing and excellent fastness to water are obtained.

## Example 3

A mixed fabric of 30 per cent of wool and 70 per cent of viscose artificial silk is dyed in the manner described in Example 1 with the dyestuff 5 derived from 1 molecular proportion of tetraazotized 4,4'-diaminodiphenyl, 1 molecular proportion of salicylic acid and 1 molecular proportion of a 2- (paracresotinsulphonyl) - amino - 5 - hydroxynaphthalene-7-sulphonic acid (coupled alkaline) having the following formula:—



(obtainable in the following manner: 239 parts 20 of 2-amino-5-hydroxynaphthalene-7 - sulphonic acid are stirred with water, and dissolved by adding a sufficient amount of caustic soda solution. After having added 200 parts of crystallized sodium acetate, from 280 to 300 parts of p- cresotinic acid sulphochloride are introduced in small batches while stirring at from 20 to 25° C. until the acylation is completed. The solution may then be employed for being coupled with the diazonium salt without further purification). 25 30 Yellowish red shades of bad fastness to washing and entirely insufficient fastness to water are obtained. By aftertreatment of the fabric for half an hour with 2 per cent of chromium sulphate (calculated with reference to the weight of the 35 fabric) somewhat more bluish dyeings are obtained having greatly improved fastness to washing and excellent fastness to water.

## Example 4

40 A mixed fabric of 70 per cent of wool and 30 per cent of staple fibre ("Zellwolle") is dyed according to the metachrome process with a mixture of the substantive dyestuff of the formula



50 and the dyestuff obtainable by coupling diazotized 3,4,6-trichlor-2-amino - 1 - hydroxybenzene

with 1-acetylamo - 8 - hydroxynaphthalene-4 - sulphonic acid from greenish-blue to navy blue shades being obtained. By treating the fabric thus dyed in a separate bath with 2 per cent (calculated on amount of fabric) of chromifluoride, the fastness to washing, perspiration, water and fulling is remarkably improved.

5 Dyeings having similar good properties are obtained if 2 per cent of chromium sulphate are added to the metachrome bath towards the end 10 of the dyeing process and then treating the dyeing in a further bath for from 15 to 20 minutes with Marseille soap at from 40° to 50° C.

It is also possible to dye the fabric with the 15 said dyestuff mixture from a neutral or weakly acid bath, then to effect the formation of the complex chromium compound in the usual manner by adding from 2 to 3 per cent of sodium bichromate and then to aftertreat the fabric in a fresh bath with 2 per cent of chromium sulphate. 20

The dyeings obtained in the first bath may also be treated in a second bath with between 2 and 3 per cent of sodium bichromate in the presence of 2 per cent of acetic acid, and from 2 to 3 per cent of chromium sulphate.

25

What I claim is:

1. A process of dyeing mixed fabrics of animal and vegetable fibres with substantive azo dyestuffs capable of being chromed which comprises treating the fibre on which the said dyestuffs are already reacted with a salt of chromic acid, with a salt of trivalent chromium in a separate bath.

30

2. A process of dyeing mixed fabrics of animal and vegetable fibres with substantive azo dyestuffs capable of being chromed which comprises 35 treating the fibre with the said dyestuffs and first with a salt of chromic acid and in the same bath with a salt of trivalent chromium added towards the end of the treatment.

35

3. A process of dyeing mixed fabrics of animal and vegetable fibers with substantive azo dyestuffs capable of being chromed which comprises applying the dyestuffs to the fabric, treating the fabric with an aqueous solution of a chromic acid salt and then treating the fabric with a salt of trivalent chromium.

45

4. The process of claim 3, wherein the azo dyestuff applied to the fabric contains a salicylic acid radical in its molecule.

40

50 HERMANN WINKELER.